# EUROPEAN PATENT SPECIFICATION

(11) **EP 1 374 710 B1**
(45) Date of publication and mention of the grant of the patent: **19.09.2007**
(21) Application number: 03013874.7
(22) Date of filing: 19.06.2003
(51) Int. Cl.: A44B 1/02, A44B 1/12

(54) **Buttons that can be dyed with the fabrics they are sewn upon**
Knöpfe die zusammen mit ihrem Gewebetrager färbbar sind
Boutons pouvant être teints avec leur support en tissus

(30) Priority: 24.06.2002 IT MI20021387
(43) Date of publication of application: 02.01.2004
(73) Proprietor: Bottonificio Lariano S.r.l., 22073 Fino Mornasco (Como) (IT)
(72) Inventor: Zanini, Battista, 22073 Fino Mornasco (Como) (IT)
(74) Representative: Lecce, Giovanni

(56) References cited:
- WO-A-96/11793
- GB-A- 560 297
- GB-A- 191 128 297

## Description

The present invention refers to the manufacturing of buttons that can be dyed with the fabrics they are sewn upon.

It is known that one of the greatest problems concerning the ready-to-wear monochrome garments is that after their making-up with coarse fabric, they must be sent to the dyeing factories to be dyed with the required colours and they must come back to the making-up departments so that the buttons can be sewn.

These needs require the presence of people and transport means, longer working times, increase in times and production costs in order to prepare the material, the handling of the made-up coarse garments to and from the dyeing factories for the finishing and the sewing of the buttons.

GB 28297 A.D.1911 discloses a parchment button that can be dyed with the fabric to which it is sewn, obtained by uniting together several webs of parchment, stamping the resulting web into discs that are pressed and drilled to obtain the desired finished button. No suggestion is given to improve the properties of the parchment paper to receive and maintain the dye.

Objects of the present invention are to remove the above-mentioned drawbacks and to generally improve the button capability to receive and maintain the die. The invention accomplishes the above objects through a process as claimed in claim 1. The buttons obtained through the process according to the invention are made of material having features similar to the ones of the fabrics; the coarse buttons, that are not dyed, are sewn on garments at the end of their making-up with coarse fabrics; the coarse garments complete with the coarse buttons, are sent to the dyeing factories and submitted to the simultaneous dyeing with the treatment the fabrics are usually submitted to.

The advantages obtained by the present invention essentially consist in the fact that the vegetable similar materials the fabrics and correspondent buttons are made of, allow the simultaneous dyeing thus assuring an even dyeing both for type, hue, intensity, consistency and duration.

The invention is described in detail here below, according to examples showing the procedure to obtain some buttons and their dyeing at the same time as the fabrics that are given only by way of non-limitative example.

The vegetable fibre pulp is treated under pressure (at about 1800÷2500 kg/cm² depending on the mechanical features and on the thickness of the buttons to be produced) in order to obtain single-layer or multi-layer plates with different thickness and appropriate physical features in order to assure the required resistance and mechanical workability of the buttons.

The pressed vegetable pulp plates, in particular the pressed plates obtained by cellulose fibres (white fibrous polysaccharide component of the cellular part of vegetables) are then submitted at least to one targeted cleaning treatment in order to remove the natural wastes contained therein.

These treatments aim at obtaining the utmost pureness of the material.

One of the cleaning treatments consists in:
- putting the vegetable fibre pulp plates in a solution with a 1/5÷1/10 ratio of water with PH 5.5÷9 and detergent in a 3÷8 cc/I ratio of water at the temperature of 40÷60°C for a variable time of about 0.5÷1.5 hours,
- carrying out a first rinsing in movement at about 70÷100 °C for a variable time of about 5÷15 minutes in an aqueous solution with 3÷9 gr/l of detergent,
- carrying out a second rinsing only in water.

As a non-limitative example, the physical features obtained on the pressed vegetable fibre pulp plates submitted to the above-mentioned cleaning procedure are the following ones: density: 0.8÷1.8 g/cm³, water absorption 3÷22%, humidity coefficient 5=12%, compression resistance 137.29 ÷ 294.19 MPa (14÷30 kgF/mm²), bending resistance 127.48 ÷ 147.09 MPa (12÷25Jgf.mm²), resistance to shocks 294.19 ÷ 490.33 N (30÷50kgFcm/cm), elastic modulus about (29.42÷78,45) E+01x0⁴ (3÷8x10.4 kgF/cm²), hardness 70÷ 120 Rockwell.

Through workings with laser cut some disks or washers of the required sizes are obtained and

Then turned and/or machine worked with the usual techniques in order to obtain buttons having the required sizes, shapes and pass-through holes for the sewing yarns. The finished buttons are then submitted to a finishing process with a second and even surface cleaning to be prepared for the dyeing consisting in:
- an aqueous solution bath about 40÷60g/l of caustic soda or similar product, a 1.62÷1.45 kg/dm³; 30-45° Baumè for a variable time of about 1.5÷3.0 hours,
- a first warm rinsing,
- a first neutralizing treatment for a variable time of about 10÷30 minutes, with 2÷10 cc/l of glacial acid at 30÷60°C,
- a second warm rinsing,
- a cold rinsing with centrifugation,
- drying in a convection oven.

The worked buttons made of completely purified cellulose pulp are substantially white or white/ivory and have inner features corresponding to the white or white/ivory colour and to the inner ones of the coarse linen and/or cotton yarns for the manufacturing of fabrics that are especially used to make-up monochrome garments.

The correspondent vegetable fibre buttons obtained by the above mentioned procedure are sewn on said coarse garments thus obtaining similar and homogeneous fabric-button combinations that can be submitted to simultaneous dyeing, in the same baths with the same procedures, sequences and treatment times that have been adopted up to now for the fabrics without buttons.

The dyes obtained on buttons with any dyeing bath or monochrome colour hue, are perfectly identical to the ones obtained on the fabrics the buttons are to be sewn upon.

Even though the present invention has been described according to procedures and treatments that are given only by way of non-limitative example, it is clear that various changes to the compositions, procedure sequences, treatments and combinations of methods, clearing and neutralizing products can be carried out by people skilled in the art without leaving its purpose and protection scope.

## Claims

1. A process for manufacturing buttons, comprising the steps of:
- treating under pressure a pulp of cellulose fibres to obtain a single or multi-layer plate;
- subjecting said plate to a first cleaning treatment to remove the natural wastes contained therein;
- forming disks or washers from said plates through laser cut;
- machining said disks or washers to obtain buttons having the required sizes, shapes and pass-through holes for the sewing yarns;
- submitting said buttons to a finishing process comprising a second cleaning to prepare the buttons to being dyed together with the fabric to which they will be sewn.

2. A process as claimed in claim 1, **characterised in that** said first cleaning treatment comprises:
- putting the vegetable fibre pulp plates in a solution with a 1/5-1/10 ratio of water with PH 5.5-9 and detergent in a 3-8 cc/l ratio of water at the temperature of 40-60°C for a variable time of about 0.5-1.5 hours,
- carrying out a first rinsing in movement at about 70-100°C for a variable time of about 5-15 minutes in an aqueous solution with 3÷9 gr/I of detergent,
- carrying out a second rinsing only in water.

3. A process as claimed in claim 2, **characterised in that** after said first cleaning treatment, the pressed vegetable fibre pulp plates exhibit the following properties: density: 0.8-1.8 g/cm³, elastic modulus about (29.42 - 78,45) E+01x10⁴ (3-8×10.4 kgF/cm²), hardness 70-120 Rockwell.

4. A process as claimed in claim 2 or 3, **characterised in that** said second cleaning treatment comprises subjecting the buttons to:
- an aqueous solution bath about 40-60g/l of caustic soda, a 1.62-1.45 kg/dm³ (30-45° Baumè) for a variable time of about 1.5-3.0 hours,
- a first warm rinsing,
- a first neutralizing treatment for a variable time of about 10-30 minutes, with 2-10 cc/l of glacial acid at 30-60°C,
- a second warm rinsing,
- a cold rinsing with centrifugation,
- drying in a convection oven.

5. A process as claimed in claim 1, **characterised in that** said single or multi-layer plate is obtained by treating a pulp of cellulose fibres under a pressure of about 1800-2500 kg/cm².

## Patentansprüche

1. Verfahren zur Herstellung von Knöpfen, umfassend die Schritte:
- Behandeln einer Pulpe von Cellulosefasern unter Druck, um eine Einzel- oder Mehrschichttafel zu erhalten;
- Unterziehen der Tafel einer ersten Reinigungsbehandlung, um die darin enthaltenen natürlichen Verunreinigungen zu entfernen;
- Ausbilden von Platten oder Scheiben aus den Tafeln durch Laserschneiden;
- Bearbeiten der Platten oder Scheiben, um Knöpfe mit den erforderlichen Größen, Formen und Durchgangsöffnungen für das Vernähen von Garnen zu erhalten;
- Unterziehen der Knöpfe einer Abschlussverarbeitung umfassend ein zweites Reinigen, um die Knöpfe dahingehend vorzubereiten, zusammen mit dem Stoff gefärbt zu werden, an welchen diese genäht werden.

2. Verfahren nach Anspruch 1, **dadurch gekennzeichnet, dass** die erste Reinigungsbehandlung umfasst:
- Legen der Pflanzenfaserpulpentafeln in eine Lösung mit einem 1/5-1/10-Verhältnis von Wasser mit pH 5,5-9 und einer Detergenz in einem 3-8 ccm/l-Verhältnis von Wasser bei der Temperatur von 40-60°C für eine variable Zeit von etwa 0,5-1,5 Stunden,
- Ausführen eines ersten Spülens in Bewegung bei etwa 70-100°C für eine variable Zeit von etwa 5-15 Minuten in einer wässrigen Lösung mit 3-9 gr/l von Detergenz,
- Ausführen eines zweiten Spülens nur in Wasser.

3. Verfahren gemäß Anspruch 2, **dadurch gekennzeichnet, dass** nach der ersten Reinigungsbehandlung die gepressten Pflanzenfaserpulpentafeln die folgenden Eigenschaften zeigen: Dichte: 0,8-1,8 g/cm³, Elastizitätsmodul etwa (29,42-78,45) E+01x10⁴ (3-8x10,4 kgF/cm²), Härte 70-120 Rockwell.

4. Verfahren gemäß Anspruch 2 oder 3, **dadurch gekennzeichnet, dass** die zweite Reinigungsbehandlung ein Unterziehen der Knöpfe wie folgt umfasst:
- ein Bad in wässriger Lösung von etwa 40-60 g/l von Natronlauge, 1,62-1,45 kg/dm³ (30-45° Baumè) für eine variable Zeit von etwa 1,5-3,0 Stunden,
- ein erstes warmes Spülen,
- eine erste Neutralisierungsbehandlung für eine variable Zeit von etwa 10-30 Minuten mit 2-10 ccm/l von Eisessig mit 30-60°C,
- ein zweites warmes Spülen,
- ein kaltes Spülen mit Zentrifugation,
- Trocknen in einem Konvektionsofen.

5. Verfahren gemäß Anspruch 1, **dadurch gekennzeichnet, dass** die Einzel- oder Mehrschichttafel durch Behandeln einer Pulpe von Cellulosefasern unter einem Druck von etwa 1800-2500 kg/cm² erhalten wird.

## Revendications

1. Procédé de fabrication de boutons, comprenant les étapes consistant à:
- traiter sous pression une pulpe de fibres de cellulose pour obtenir une plaque à couche unique ou à couches multiples;
- soumettre ladite plaque à un premier traitement de nettoyage pour enlever les rebuts naturels qui y sont contenus;
- former des disques ou des rondelles à partir desdites plaques par coupe par laser;
- usiner lesdits disques ou rondelles pour obtenir des boutons présentant les dimensions, configurations et orifices traversants requis pour les fils de couture;
- soumettre lesdits boutons à un processus de finition comprenant un deuxième nettoyage pour préparer les boutons qui sont à teindre en commun avec l'étoffe à laquelle ils seront cousus.

2. Procédé selon la revendication 1, **caractérisé en ce que** ledit premier traitement de nettoyage comprend les étapes consistant à:
- mettre les plaques de pulpe de fibres végétales dans une solution aqueuse à une teneur de 1/5 à 1/10 rapportée à l'eau, à pH de 5,5 à 9, avec un détergent à une teneur de 3 à 8 cc/l d'eau, à la température de 40 à 60 °C, pendant un temps variable d'environ 0,5 à 1,5 heures,
- exécuter un premier rinçage en mouvement à environ 70 à 100 °C pendant un temps variable d'environ 5 à 15 minutes dans une solution aqueuse à teneur de 3 à 9 g/l de détergent,
- exécuter un deuxième rinçage à l'eau seulement.

3. Procédé selon la revendication 2, **caractérisé en ce que** les propriétés des plaques comprimées de pulpe de fibres végétales, après le premier traitement de nettoyage, sont les suivantes: densité: 0,8 à 1,8 g/cm³, module d'élasticité environ (29,42 à 78,45) E+01x10⁴ (3 à 8 x 10.4 kgF/cm²), dureté Rockwell: 70 à 120.

4. Procédé selon la revendication 2 ou 3, **caractérisé en ce que** ledit deuxième traitement de nettoyage comprend les étapes consistant à soumettre les boutons à:
- un bain de solution aqueuse d'environ 40 à 60 g/l de soude caustique, à 1,62 à 1,45 kg/dm³ (30 à 45 ° Baumé) pendant un temps variable d'environ 1,5 à 3,0 heures,
- un premier rinçage à chaud,
- un premier traitement de neutralisation, pendant un temps variable d'environ 10 à 30 minutes au moyen de 2 à 10 cc/l d'acide acétique glacial à 30 à 60 °C,
- un deuxième rinçage à chaud,
- un rinçage à froid avec centrifugation,
- un séchage en four à convexion.

5. Procédé selon la revendication 1, **caractérisé en ce que** ladite plaque à couche unique ou à couches multiples est obtenue en traitant une pulpe de fibres de cellulose sous une pression de 1.800 à 2.500 kg/cm².
